

## UNITED STATES PATENT OFFICE

2,455,659

## OILY COMPOSITION

Gordon W. Duncan, Westfield, and John C. Zimmer, Union, N. J., assignors to Standard Oil Development Company, a corporation of Delaware

No Drawing. Application October 5, 1945,  
Serial No. 620,630

1 Claim. (Cl. 252—33)

**1** The present invention relates to a method of producing improved oily compositions which may be used for many purposes, and especially to improvements in such oils by giving to them greater ability to protect metals, with which they are in contact, from corrosion caused by contamination of the oily composition with moisture. The invention contemplates not only the method of producing the oils, but the new compositions themselves.

Various soluble oils are known to the arts and they are used for many purposes such as for lubricating and cooling in the cutting and grinding of metals. These compositions are normally supplied by the manufacturers as oils and are diluted with water by the operator before use. The compositions generally contain an oily vehicle, either mineral or fatty oil, together with an emulsifier which brings about the formation of the emulsion when water is added.

Other types of oil compositions such as slushing oils and greases are not designed for solubilizing but are employed, on the other hand, to submerge or cover metal surfaces during long periods of storage and to protect them from corrosion, spotting, staining and discoloration. Such corrosive action is usually due to the action of the atmosphere and/or moisture therein and the purpose of the anti-corrosive compound is to prevent deterioration under these influences. Nevertheless, in many cases, oils do permit a minor form of spotting or discoloring and the object of the present invention is to remove this deficiency.

Still other oils are employed for general or specific lubrication purposes and as hydraulic media, and in many such cases it is necessary or desirable to fortify the oil to an extremely high degree against staining and spotting of metal surfaces caused by water contamination of the oils.

The present invention deals with the improvement of all such oils in this particular direction. It is also highly desirable that these oils should be clear, free from any sediment and otherwise suited to the intended purpose.

In making the present compositions, it will be understood from what has been said before that there is an oily vehicle which comprises the major portion of the present composition. This may be an oil of vegetable, animal or mineral origin. The common fatty oils such as castor oil, lard oil and the like may, of course, be used but the hydrocarbon oils are particularly to be desired, whether they are derived from asphaltic, mixed base or paraffinic crudes, and the oil must be

selected with a view to the particular use intended, that is to say, its flash point, viscosity and the like must be adapted to the particular use, just as it is done at the present time.

**2** To this oil base is then added from 0.05 to 10.0%, depending upon contemplated use of the product, of an oil-soluble sulfonate salt which is well known to the petroleum art and is obtained as a by-product in the refining of mineral oils, particularly lubricating oils, with concentrated or fuming sulfuric acid. Alkali and alkaline earth metal sulfonates are normally preferred but other metal and nitrogen base sulfonates may be employed. The particular sulfonate is of the type generally known as "M" soap or "mahogany" soap and is also known as the oil-soluble sulfonate to distinguish it from the so-called "green" acid soaps which are water-soluble. It is usually available as a 30 to 70% concentrate in lubricating oil. This material is obtainable in several different grades of purity and derived from several kinds and viscosities of oil so that the grade employed should be chosen in view of the particular use.

The third ingredient of the present composition is an inorganic salt which is possessed of corrosion inhibiting properties when dissolved in water. Various inorganic salts of this type are known but the principal ones to be mentioned here are borax, sodium tetra pyrophosphate, sodium carbonate, sodium chromate, sodium arsenite and especially sodium nitrite. These salts are all water soluble but are not normally soluble in oil, and the purpose of the invention is to stably incorporate them in the oil. The invention is carried out in the following manner:

An aqueous solution of the inorganic compound is added to the sulfonate oil concentrate and emulsified therewith by agitation. The concentration of the salt in the water phase is not critical, but the ratio of the inorganic compound to the sulfonate should, in all cases, be such that there is present at least a mol equivalent of the sulfonate salt for each mol equivalent of the inorganic salt. If desired, more of the sulfonate may be employed and in many cases it may be desirable to employ as high as 4 mols of sulfonate per mol of inorganic material.

After the emulsion is formed, it is heated carefully with agitation to effect the vaporization of the water from the emulsion. This may be accomplished in open kettles or evaporators or other equipment designed for the purpose and, as the water is removed, the inorganic material becomes thoroughly incorporated in the sulfonate concentrate, which remains in a homogeneous

condition. Excessive foaming during this operation may be controlled by the addition of a known defoaming agent, e. g., an organic silicone polymer. The inorganic salt appears to be quite stably incorporated in the form of a complex and it does not settle out or precipitate while stored under normal conditions. It will be noted that in many instances the inorganic salt has a pronounced thinning action on the sulfonate concentrate. This is illustrated by a reduction in viscosity of a 50% sodium sulfonate concentrate from 660 to 290 Saybolt Universal seconds (at 210° F.) by the addition of 1.8% sodium nitrite.

This concentrate can now be added to the oil base as desired along with other constituents normally employed in an oil designed for the particular purpose. Such other constituents include oxidation inhibitors, dyes, perfumes, oiliness agents, E. P. agents, emulsifiers, detergents, pour depressants, V. I. improvers, organic bases, soaps, thickeners, coupling agents, or other ingredients as desired. The composition is then in condition for shipping to the ultimate consumer.

The action of the sulfonate in effecting the solubility of a normally insoluble inorganic salt is not clearly understood. It may be due to the formation of a mixed salt of the sulfonate and the inorganic acid but the explanation may be quite otherwise. It is sufficient here merely to recite the facts. To illustrate further the present composition and its use, the following examples may be considered:

#### EXAMPLE I

A petroleum sulfonate-inorganic corrosion inhibitor complex suitable for use in compositions of this invention was prepared as follows: 1000 grams of a 50% solution of 450 molecular weight petroleum sodium sulfonates in a paraffinic oil of 100 SUS viscosity (at 100° F.) was emulsified at 120° F. with 125 grams of a solution consisting of 25 grams of commercial grade sodium nitrite and 100 grams of distilled water. One drop of an organic silicone polymer was added to control foaming and the emulsion heated to 300° F. to remove the water by evaporation. The resultant product (containing 2.5% sodium nitrite) was clear, stable to storage, and appreciably more fluid than the original.

#### EXAMPLE II

When a soluble oil is diluted with water by the ultimate user, a stable emulsion is formed which can be employed as a metal working lubricant as mentioned above. Although satisfactory for the intended purpose this emulsion may cause serious corrosion of the machined parts, tools, and machinery. As an example of the effectiveness of compositions of our invention, the following may be cited:

A soluble cutting oil was prepared according to the following formula:

#### Soluble cutting oil

| Ingredient                             | Per Cent by Weight |
|----------------------------------------|--------------------|
| Pale Oil, 100 SUS viscosity at 100° F. | 75.55              |
| 50% sodium petroleum sulfonate in oil  | 19.00              |
| Naphthenic Acid                        | 2.50               |
| Caustic Soda                           | 0.40               |
| Isopropyl Alcohol                      | 0.90               |
| Water                                  | 1.60               |
| Carnauba Wax                           | 0.05               |

Emulsions of this oil were then compared with

those of an oil of the same composition prepared with the product of Example I, replacing the simple sulfonate concentrate used above with the concentrate containing sodium nitrite. In the test employed a 10% emulsion of the oil in water was poured through malleable iron filings contained in a Gooch crucible. After 24 hours the degree of corrosion was rated on a scale of 0 for no corrosion to 5 for complete rusting. The following data were obtained:

#### Gooch crucible corrosion test (malleable iron filings)

| 15 | Emulsion                              | Corrosion Rating     |      |
|----|---------------------------------------|----------------------|------|
|    |                                       | Water/oil Ratio 25/1 | 50/1 |
| 20 | Soluble oil                           | 1                    | 2-3  |
|    | Soluble oil containing sodium nitrite | 0                    | 0-1  |

These data indicate that the soluble oil containing sodium nitrite is much more resistant to rusting than the oil which does not contain the inorganic inhibitor.

#### EXAMPLE III

The lubricating systems of many different types of machinery frequently are contaminated with water, introduced either by condensation or by admixture of water or aqueous solutions from various sources. Although many different agents, including petroleum sulfonates, are effective in enabling the lubricating oil to prevent corrosion of vertical and sloping surfaces, these are not very effective when the water lies on a horizontal surface, such as the bottom of an oil sump or in various bearings and other parts of the system. We have now found that such oils are satisfactorily resistant under these conditions if the sulfonate contains a suitable inorganic inhibitor such as sodium nitrite, sodium chromate, sodium arsenite or materials which act in a similar manner. This property may be evaluated by the Naval Research Laboratory "Static drop test" in which a drop of water is placed on a steel specimen immersed in the oil at 160° F. for 7 days. As shown by the following data, the materials of our invention show considerable superiority in this test.

#### Naval research laboratory static drop test @ 160° F.

[Test oil: Highly refined paraffinic oil of 43 S. U. S. viscosity at 210° F.]

| 55 | Additive                                                                                     | Time to Initial Rusting |                    |
|----|----------------------------------------------------------------------------------------------|-------------------------|--------------------|
|    |                                                                                              | 1 hour.                 | 1 day.             |
| 60 | 1 None                                                                                       |                         |                    |
|    | 2 0.05% zinc naphthenate + 0.2% of a 50% sodium sulfonate concentrate                        |                         | No rust at 7 days. |
|    | 3 No. 2 in which the 50% sulfonate concentrate was the product of Example I.                 |                         | 3 days.            |
|    | 4 6% of a 50% sodium sulfonate concentrate + 3% of neutral wool grease                       |                         | No rust at 7 days. |
|    | 5 No. 4 in which the sulfonate concentrate was the product from Example I.                   |                         | No rust at 7 days. |
|    | 6 No. 4 in which 2.0% of potassium arsenite was incorporated in the sulfonate concentrate    |                         | No rust at 7 days. |
|    | 7 10% of a 30% calcium sulfonate concentrate                                                 |                         | 3 days.            |
|    | 8 No. 7 in which 2% of sodium chromate was incorporated in the calcium sulfonate concentrate |                         | No rust at 7 days. |

#### Example IV

In still another example, a polished steel panel was coated with a petrolatum slushing composition (165° F. melting point) which contained

3% of a 50% concentrate of sodium sulfonate in oil, and stored for one month at 100° F. with constant moisture condensation on the panel. At the end of this time, considerable under-film corrosion had occurred. In the same test, a petro-latum containing 3% of the product of Example I afforded complete protection to the panel.

From the above examples it may be seen that our invention can be beneficially employed in the preparation of many petroleum products for use where moisture corrosion of metal surfaces is a problem. We contemplate its use in hydro-carbon fuels, lubricants for all purposes, slushing compositions, flushing oils, emulsifiable oils, greases, hydraulic media, etc.

We claim:

15 A composition suitable for use as a soluble cutting oil, or the like, consisting essentially of about 84% mineral base lubricating oil, about

8% sodium petroleum sulfonate, about 2.5% sodium nitrite, about 2.5% naphthenic acid, 0.4% caustic soda, 0.9% isopropyl alcohol, 0.05% wax, and a small amount of water, said proportions being by weight.

GORDON W. DUNCAN.  
JOHN C. ZIMMER.

## REFERENCES CITED

The following references are of record in the file of this patent:

## UNITED STATES PATENTS

| Number    | Name     | Date          |
|-----------|----------|---------------|
| 2,182,992 | Lebo     | Dec. 12, 1939 |
| 2,079,051 | Sullivan | May 4, 1937   |
| 2,060,110 | Paxton   | Nov. 10, 1936 |